

Patented Sept. 28, 1926.

1,601,327

# UNITED STATES PATENT OFFICE.

BELA W. ROTE, OF CLEVELAND, OHIO.

## COMPOSITE HEEL.

No Drawing.

Application filed January 20, 1922. Serial No. 530,533.

My invention relates to shoe heels and particularly to a composite half-heel or heel lift formed from tough, wear-resisting and non-slip material. This composite heel may 5 be utilized as a tread-section for a compound heel having an inner soft cushion section serving as a backing adjacent the shoe heel proper.

The following description sets forth in 10 detail certain ingredients adapted to be combined to form my improved composite shoe heel, and certain steps by which the same are combined, the disclosed proportions of said ingredients and the method of combining the same being illustrative of various proportions and steps suitable for the improved composition and the forming of the same.

I produce the stock suitable for my improved heel by the process described and 20 claimed in my pending application for U. S. Letters Patent, Serial No. 430,086. Rubber stock may be utilized for an inner cushion section. In the latter event, I 25 anchor in any suitable manner these two sections one to the other so as to produce one united mass of the whole having a homogeneous structure in and adjacent to the plane containing the joint between the 30 two sections. Preferably, I vulcanize the two sections together so as to produce this single mass. I do not limit myself as to the relative thickness of the two sections, the same being of equal thickness or one of 35 a greater or less thickness than the other, according to the particular demand to be satisfied by the composite structure.

When my improved heel composition is combined with an inner cushion section, 40 these two sections are anchored one to the other so as to produce a homogeneous structure in the plane of the joint between the two sections, this anchorage preferably being obtained by vulcanizing the two sections. This vulcanization as is known to 45 those well skilled in the art, is effected in a suitable mold. The usual washers molded in heel lifts and through which and up to which the nails are driven for securing 50 the heel to the shoe are utilized when two sections are thus combined to form a compound heel. In the event that my improved composite heel forms the whole heel structure and is not utilized with an inner rubber cushion section, I can dispense with 55 the usual washers around the nail holes

inasmuch as my composition stock is firm enough to hold the nail. This permits considerable saving in both material and labor in connection with the manufacture. In 60 so far as I am advised practically all rubber heel lifts require the washers around the nail holes and it is common practice to utilize the same.

Briefly now I shall describe the process 65 of producing the tough wear-resisting composite heel, which process is described and claimed in said application, Serial No. 430,086. I first dissolve a minor portion of rubber in benzol or its equivalent. One example 70 of such equivalent is gasoline of seventy (70) Baumé or over. I then saturate a major portion of cotton or its equivalent with the rubber solution. This cotton is any suitable 75 fibre material essentially wear-resisting and non-elastic, the particular grade of the same depending upon the final product which is desired, and it may be cotton fibre, of a high or low order, or waste or scrap leather, or waste or scrap jute, or a combination of 80 the same. Also dependent upon the final product desired, the rubber may be pure Pará or smoked sheets, which is a refined rubber, or crepe which is plantation rubber and less dense than sheets, or coarse rubber 85 which is a second or third grade raw rubber, or reclaimed rubber, which is any grade being subjected to its second or third use. By a minor portion of rubber, I mean substantially one part by weight to four parts of 90 the fibre or its equivalent. The mixture of rubber and cotton is dried thoroughly of the contained moisture, this drying being preferably effected by a vacuum drying process. The heat to which the vacuum drier 95 is subjected will vary according to the heat that is allowed for the drying. The dried product is then warmed and compressed, preferably by rolls, filling, pigment and vulcanizing material being added during the 100 pressing or rolling operation. These last-mentioned materials are added also in a minor portion, the aggregate of the same being substantially by weight equal to the weight of the rubber.

Dependent upon the nature of the desired product, the filling, pigment and vulcanizing material will vary both as to its ingredients and the relative proportions of the same. For instance, suppose seventy (70) parts of 110 cotton or its equivalent to have been utilized and fifteen (15) parts of pure Pará rubber,

the filling, pigment and vulcanizing material would consist of five (5) parts litharge, five (5) parts of magnesia, three (3) parts of gloss black or lamp black, and two (2) parts pure sulphur. These ingredients will produce a high grade black wear-resisting and non-slip plastic composition suitable for manufacturing a high grade leather substitute. Again, supposing a high grade leather substitute of tan color is desired. Suitable ingredients would be sixty-five (65) per cent cotton fibre of high order, substantially fifteen (15) per cent pure Pará rubber, substantially five (5) per cent magnesia, substantially five (5) per cent oxy-sulphide of antimony or red antimony, substantially five (5) per cent zinc oxide, substantially three (3) per cent petrolatum and substantially two (2) per cent sulphur. The magnesia, besides serving as a filler, allows increased heat under vulcanizing, because it is not greatly affected by the heat, the antimony serves as a pigment, the zinc oxide serves as a filler and also assists in the vulcanization. The petrolatum serves as binding material and the sulphur assists greatly, of course, in the vulcanization. After the filling, pigment and vulcanizing material has been compressed and rolled into the cotton-rubber mixture, as above mentioned, the resultant product is sheeted to the desired

thickness and cured in a flat plate vulcanizing press.

From the sheeted artificial leather, produced as above described, are stamped my improved composite heels or lifts adapted to serve as the tread sections of heel and, in the latter event, to these sections are anchored soft cushion sections, preferably of rubber, by any suitable process, preferably by vulcanizing the two sections together in a suitable mold. This anchorage would be increased by any indentations or unevenness in the contacting surfaces of the two sections.

What I claim is:—

1. A composite heel comprising, a leather substitute section composed of substantially seventy (70) parts cotton fibre, fifteen (15) parts vulcanized pure Pará rubber, and thirteen (13) to eighteen (18) parts filling and pigment.

2. A composite heel comprising, a leather substitute tread section composed of substantially seventy (70) parts cotton fibre, fifteen (15) parts pure Pará rubber, five (5) parts litharge, five (5) parts magnesia, three (3) parts gloss black and two (2) parts pure sulphur.

Signed by me this 14th day of December, 1921.

BELA W. ROTE.